

## UNITED STATES PATENT OFFICE

2,421,004

## MINERAL OIL COMPOSITION

Henry G. Berger, Glen Rock, and Everett W. Fuller, Woodbury, N. J., assignors to Secony-Vacuum Oil Company Incorporated, a corporation of New York

No Drawing. Application August 3, 1944.  
Serial No. 547,981

11 Claims. (Cl. 252—33.4)

1

This invention has to do with a new and novel mineral oil composition and, more particularly, has to do with a mineral oil composition containing minor proportions of an oil-soluble detergent and of an oil-soluble, phosphorus- and sulfur-containing reaction product.

It is well known to those familiar with the art that mineral oils are generally characterized by one or more undesirable characteristics which limit their use. One such characteristic is their instability under operating conditions normally encountered in present-day engines, such that after a relatively short time, metal engine parts become contaminated with sludge, lacquer and resinous materials. In many instances, the said materials form in and about piston rings causing them to stick, the phenomenon being referred to as "ring-sticking." As a consequence of the instability of the oil, engine operating efficiency is seriously reduced. Another undesirable characteristic of mineral oils is their tendency to oxidize whereupon acidic materials are formed. These acidic materials corrode metal engine parts, particularly alloy bearings such as those of the copper-silver, copper-lead, etc., type.

It is also well known in the art that numerous materials have been proposed as improving or fortifying agents for use in mineral oils to counteract or retard the aforesaid undesirable characteristics. Of the improving agents previously proposed, oil-soluble metal sulfonates have been found to be satisfactory in imparting detergent properties to mineral oil. Unfortunately, however, such sulfonates fail to improve, and in some cases even impair, other characteristics of mineral oils. In some instances, for example, metal sulfonates have increased the formation of acidic materials in mineral oils during use, thus inducing corrosion of metal parts with which the oils come in contact.

It has now been found that the corrosion and oxidation characteristics of an oil containing a small amount of an oil-soluble metal sulfonate can be greatly improved by incorporating therewith a small amount of an oil-soluble phosphorus- and sulfur-containing reaction product of phosphorus pentasulfide and a cycle stock characterized by an olefin and an aromatic content of from about 3 per cent to about 7 per cent and from about 40 per cent to about 60 per cent, respectively. More specifically, it has been found that an extremely stable oil having outstanding detergent, oxidation and corrosion characteristics is obtained by incorporating in an oil containing a metal sulfonate, a small amount

5 of a reaction product of the aforesaid type. It has also been found that oils similarly characterized are obtained by incorporating a small amount of the said reaction product into oils containing small amounts of oil-soluble salts of organic acids, which possess detergent properties.

All oil-soluble metal sulfonates are contemplated herein, typical of which are those obtained from aromatic hydrocarbons or substituted aromatic hydrocarbons, and a sulfonating agent such as strong sulfuric acid, oleum, chlorosulfonic acid and the like. Other typical sulfonates are those obtained by treatment of paraffins, naphthenes and various petroleum fractions—paraffinic, naphthenic or aromatic—with the same reagents. Preferred, however, are the metal salts of sulfonic acids of wax-substituted benzene and wax-substituted naphthalene wherein the wax substituent is a long-chain aliphatic hydrocarbon group containing at least about 18 carbon atoms and is obtained from paraffin wax.

10 All metals are contemplated herein as constituents of the said metal sulfonates. Especially suitable, however, are sodium, barium and zinc. 15 It is to be understood that when the metal substituent is polyvalent, basic as well as neutral metal sulfonates are obtained and serve the purposes of this invention. Typical and preferred sulfonates are the sodium, basic calcium, basic 20 barium, neutral barium, zinc and dibasic aluminum salts of diwax-benzene sulfonate. Several such materials are described in further detail hereinafter in the examples.

25 As indicated hereinabove, oils containing other detergents—oil-soluble salts of organic acids possessing cleansing or detergent action in oil—are also substantially improved in character when a small amount of the aforesaid oil-soluble, phosphorus- and sulfur-containing reaction product 30 of phosphorus pentasulfide and a cycle stock is incorporated therein. Typical oil detergents contemplated herein are metal salts of carboxylic acids, as a calcium salt of an alkylated salicylic acid; metal salts of hydroxyaromatic carboxylic acids, as a barium phenate-carboxylate of an alkyl-substituted phenol carboxylic acid; sulfides of metal salts of hydroxyaromatic carboxylic acids, as a barium phenate-carboxylate of an alkyl-substituted phenol carboxylic acid disulfide; 35 metal salts of acid esters, as vanadyl oleyl phthalate; etc. Oil-soluble salts of organic acids such as the foregoing typical salts are well known in the art and may be prepared by any suitable method.

40 The oil-soluble, phosphorus- and sulfur-con-

2

taining reaction products contemplated herein are those obtained by reacting  $P_2S_5$  and a cycle stock, as defined above, under the following interrelated reaction conditions:

1. Between about 1 per cent and about 8 per cent by weight of  $P_2S_5$  based upon the weight of said cycle stock,
2. A temperature between about  $125^\circ C.$  and about  $200^\circ C.$ , and
3. A relatively short reaction time.

The hydrocarbon reactants are, as indicated above, cycle stocks containing from about 3 per cent to about 7 per cent of olefins and from about 40 per cent to about 60 per cent of aromatics, as determined by the following test method:

Twenty-five milliliters of a solution containing 70 per cent by weight of sulfuric acid (sp. gr. 1.84) and 30 per cent of  $P_2O_5$  are placed in a glass stoppered sulfonation bottle (a modified Babcock bottle—A. S. T. M. Standards on Petroleum Products and Lubricants, September 1943, page 381). The bottle is immersed in ice water for five minutes; then 10 milliliters of the hydrocarbon are added. The bottle is shaken for ten minutes while cooling with ice water. Sulfuric acid (sp. gr. 1.84) is added until the top meniscus of the hydrocarbon layer is brought up to the 100 per cent mark of the graduated portion of the neck. The bottle is then stoppered and is centrifuged for ten minutes. The milliliters of hydrocarbon oil layer remaining are read and this value is subtracted from the original 10 milliliters to obtain the combined amounts of aromatic and olefin contents of the sample. By repeating the same procedure, except for using 85 per cent sulfuric acid instead of the  $H_2SO_4-P_2O_5$  mixture, the olefinic content of the sample is obtained. Thus, olefinic content subtracted from the combined olefin and aromatic content gives the amount of aromatic material present.

Preferably, the hydrocarbon reactants are also characterized by the following: boiling range from about  $90^\circ C.$  to about  $400^\circ C.$  and specific gravity from about 0.88 to about 0.93. In general, such cycle stocks are obtained from thermal cracking operations of crude oils; but other stocks characterized as above may also be used. Typical of such other stocks are light gas oils, such as a light gas oil containing 4 per cent olefins and 46 per cent aromatics, a specific gravity of 0.8833 and a boiling range from  $150^\circ C.$  to  $380^\circ C.$  For this reason, the hydrocarbon reactants may be broadly considered as hydrocarbon stocks characterized by the aforesaid percentages of olefins and aromatics.

The amount of  $P_2S_5$  reacted with the cycle stocks contemplated herein is an important consideration. Stable oil-soluble reaction products containing appreciable quantities of phosphorus and sulfur are obtained when the amount of  $P_2S_5$  so reacted is from about 1 per cent to about 8 per cent by weight of the hydrocarbon reactant. Particularly preferred reaction products, however, are obtained with about 5 per cent by weight of  $P_2S_5$ . When amounts of the order of 10 per cent and 15 per cent of  $P_2S_5$  are used, it has been found that the phosphorus- and sulfur-containing reaction products obtained therewith are unstable when heated and are oil-insoluble. As used herein the term "oil soluble" is descriptive of those reaction products which are soluble in oil in amounts of at least 1 per cent by weight.

Another important consideration in the prep-

aration of the aforesaid reaction products is reaction time. In general, superior reaction products, in quantities such as shown in the following examples, are obtained when the reaction time is relatively short, such as from about 2 hours to about 8 hours. While reaction times as long as about 12 hours have been used and satisfactory reaction products obtained therewith, reaction times in the neighborhood of 4 hours are preferred. It is to be understood, however, that the reaction time may be varied considerably depending upon the quantities of reactants and the reaction temperatures used in the preparation of said reaction products.

15 The interrelation of the foregoing reaction factors will be apparent from the following typical examples recited below, and also those set forth in Table I.

#### EXAMPLE 1

20 A reaction stock—recycle stock A—from a thermal liquid phase cracking operation and having the following characteristics, was used:

|                                |          |        |
|--------------------------------|----------|--------|
| Olefin content                 | per cent | 6      |
| Aromatic content               | do       | 47     |
| Specific gravity               |          | 0.8939 |
| Aniline number                 |          | 105.5  |
| Boiling range ( $^\circ C.$ ): |          |        |
| Initial B. Pt.                 |          | 97     |
| 30 10%                         |          | 230    |
| 50%                            |          | 274    |
| 90%                            |          | 327    |
| End point                      |          | 366    |
| Recovery                       | per cent | 98.5   |

35 One thousand parts by weight of recycle stock A was reacted with stirring, with 70 parts of  $P_2S_5$  at  $180^\circ C.$  for 8 hours. The reaction mixture thus obtained was diluted with naphtha (boiling range  $88-135^\circ C.$ ), washed with 20%  $Na_2S$  solution, water washed, filtered and the filtrate heated to  $150^\circ C.$  at 10 mm. pressure to remove the naphtha. The reaction product contained 1.19% phosphorus and 3.06% sulfur, and is identified hereinafter as Product One.

#### EXAMPLE 2

40 One thousand parts by weight of recycle stock A was reacted, with stirring, with 50 parts of  $P_2S_5$  at  $150^\circ C.$  for 8 hours. The reaction mixture so obtained was then cooled to  $100^\circ C.$ , 52.5 parts (5% by weight) of Attapulgus clay were added thereto and the clay was subsequently removed therefrom by filtering. The reaction product—Product Two—contained 1.26% phosphorus and 3.6% sulfur.

#### EXAMPLE 3

45 Five hundred parts by weight of Product Two obtained in Example 2 were vacuum distilled to a maximum temperature of  $172^\circ C.$  at 3 mm. in order to remove unreacted recycle stock therefrom. The residue—Product Three—contained 3.34% phosphorus and 7.9% sulfur.

50 Reaction products obtained from recycle stock A and prepared as in Example 2 above are shown in Table I below in order to demonstrate the influence of each of the several reaction variables—time, temperature and concentration of  $P_2S_5$ . The copper strip tests referred to in the table were made by immersing a polished copper strip in a 1% blend of a reaction product in oil and heating the blend at  $100^\circ C.$  for 24 hours. The copper strip test indicates the presence or absence of free or active sulfur which corrodes copper. An asterisk (\*) has been used in the table wherever

the copper strip used in the copper strip test was not corroded in each test; that the reaction product was stable; and that the reaction product was soluble in oil.

atoms to the molecule and a melting point of 126° F. was chlorinated at about 95° C. with chlorine gas until the weight of the wax had increased about 10%. The chlorowax (10% Cl) thus ob-

Table I

|                                        | Product | P <sub>2</sub> S <sub>5</sub> ,<br>per cent<br>by wt. | Temp.,<br>° C. | Time,<br>hrs. | Composition   |               | Copper<br>Strip<br>Test | Stability | Solu-<br>bility |
|----------------------------------------|---------|-------------------------------------------------------|----------------|---------------|---------------|---------------|-------------------------|-----------|-----------------|
|                                        |         |                                                       |                |               | Per cent<br>P | Per cent<br>S |                         |           |                 |
| Temp.                                  | Four.   | 5                                                     | 150            | 4             | 1.41          | 3.4           | +                       | +         | +               |
|                                        | Five.   | 5                                                     | 190-200        | 4             | 1.23          | 3.8           | +                       | +         | +               |
|                                        | Six.    | 5                                                     | 220            | 4             |               |               | (1)                     | (2)       |                 |
| Time                                   | Four.   | 5                                                     | 150            | 4             | 1.41          | 3.4           | +                       | +         | +               |
|                                        | Seven.  | 5                                                     | 150            | 8             | 1.26          | 3.6           | +                       | +         | +               |
|                                        | Eight.  | 5                                                     | 150            | 12            | 1.2           | 3.4           | +                       | +         | +               |
| Conc. of P <sub>2</sub> S <sub>5</sub> | Nine.   | 2.5                                                   | 150            | 4             | 0.62          | 0.89          | +                       | +         | +               |
|                                        | Four.   | 5                                                     | 150            | 4             | 1.41          | 3.4           | +                       | +         | +               |

<sup>1</sup> Unstable.

<sup>2</sup> Insoluble.

It will be apparent from the data tabulated in Table I above that where a reaction temperature in excess of 200° C. was used the product is unsatisfactory. The desired reaction products as indicated in Table I are those prepared under the reaction conditions defined hereinabove.

Another cycle stock which was also found to be particularly desirable was a cycle stock, obtained from a Cross still, and characterized by the following:

|                       |               |        |
|-----------------------|---------------|--------|
| Olefin content-----   | per cent----- | 5      |
| Aromatic content----- | do-----       | 57     |
| Specific gravity----- |               | 0.9236 |
| Aniline number-----   |               | 80     |
| Boiling range-----    | ° C. 140-370  |        |

Further details regarding the character of the aforesaid reaction products may be obtained by referring to copending application Serial No. 515,418, filed December 23, 1943, of Henry G. Berger, Thomas T. Noland and Everett W. Fuller.

The oil compositions contemplated herein may also contain, in addition to an oil detergent and a cycle stock-P<sub>2</sub>S<sub>5</sub> reaction product, a small amount of one or more other oil-soluble, phosphorus- and sulfur-containing reaction products. One such reaction product is that obtained by reacting a dicyclic terpene, as pinene, and a phosphorus sulfide, as P<sub>2</sub>S<sub>5</sub>, at a temperature above about 100° C. Further details regarding the character of the said dicyclic terpene-phosphorus sulfide reaction products may be obtained by referring to copending application Serial No. 482,482, filed April 9, 1943, of Everett W. Fuller et al.

Other oil-soluble, phosphorus- and sulfur-containing reaction products which may be incorporated in the oil compositions defined above are those obtained by reaction of substantially one mol of phosphorus pentasulfide and four mols of oleyl alcohol, or oenol, at a temperature between about 125° C. and about 150° C. for a relatively short time. These reaction products are described in further detail in a copending application, Serial No. 524,490, filed February 29, 1944, of Everett W. Fuller, Henry G. Berger and Robert H. Williams.

In the following examples, typical and preferred metal sulfonates and other oil-soluble metal detergents are described in order to further explain the oil addition agents contemplated herein.

#### EXAMPLE 4

##### Basic barium diwax benzene sulfonate

A paraffin wax having an average of 24 carbon

tained was then blown with nitrogen to remove any occluded chlorine and hydrogen chloride.

One thousand and twenty parts of the above chlorowax was then reacted with 458 parts by weight of benzene in the presence of 62 parts of AlCl<sub>3</sub> at about 60° C. for about 2 hours. The excess benzene was then distilled off by warming to 115° C. with a stream of nitrogen gas bubbling through the mixture. The monowax benzene thus formed was treated with an additional 1020 parts of chlorowax and the mixture heated to 85° C. until reaction stopped. It was allowed to stand overnight at about 60° C. and then decanted from the settled AlCl<sub>3</sub> sludge and filtered. The product consisted essentially of diwax benzene.

Five thousand two hundred parts of the diwax benzene, prepared as described above, were treated with successive 250 parts of oleum, containing 15% SO<sub>3</sub>, while maintaining the temperature at 35°-50° C. After 2600 parts of oleum had been added and the reaction had ceased, 3000 parts of water were added while the mixture was thoroughly stirred. An S. A. E. 30 grade motor oil (5400 parts) was then added and the mixture was allowed to settle overnight at about 75° C. The lower layer, consisting mostly of dilute sulfuric acid, was withdrawn leaving diwax benzene sulfonic acid in the upper layer. This upper layer was treated with 3170 parts by weight of barium hydroxide octahydrate (Ba(OH)<sub>2</sub>·8H<sub>2</sub>O), which represents an excess of barium hydroxide over that required to neutralize the diwax benzene sulfonic acid and any free sulfuric acid occluded therein. The reaction mixture thus formed was heated to about 140° C. for about 6 hours with nitrogen gas bubbling through it to remove water, and it was then filtered through a layer of clay. The product—

Product A—consisted of an approximately 50% oil blend of basic barium diwax benzene sulfonate (analysis: 5.17% barium and 1.5% sulfur).

#### EXAMPLE 5

##### Basic barium diwax naphthalene sulfonate

Five hundred parts of chlorowax, containing 12% chlorine, were added to 500 parts of Stoddard solvent and 108 parts of naphthalene. The mixture was warmed to 50-60° C. and 30 grams of AlCl<sub>3</sub> were added gradually. When the reaction stopped the mixture was heated to 90° C. and blown with nitrogen gas to remove HCl. It was then allowed to stand overnight at room temperature. The lower sludge layer was removed and

the oil layer was filtered through clay. This consisted essentially of diwax naphthalene.

The diwax naphthalene was treated with 250 parts of oleum (15% SO<sub>3</sub>) by adding the latter slowly so as to keep the temperature at 40-50° C. One thousand parts of water were then added with stirring and this was followed by 500 parts of an S. A. E. 30 grade motor oil. The mixture was allowed to stand at 60-70° C. overnight and the oil layer was then withdrawn. This consisted essentially of 50% diwax naphthalene sulfonic acid in motor oil. This acid was treated with an excess of barium hydroxide and the mixture was heated to a maximum temperature of 150° C. in the presence of a stream of nitrogen to remove the water. After filtering, the Stoddard solvent was removed by heating to 170° C. at a vacuum of 5 mm. This left an approximately 50% solution of the basic barium diwax benzene sulfonate in the petroleum motor oil, which is identified as Product B. It contained 10% barium and 2.0% sulfur.

#### EXAMPLE 6

##### *Barium salt of petroleum oil sulfonate*

A Mid-Continent distillate of 95 seconds Saybolt viscosity at 100° F. was treated with oleum, the sludge was settled and removed, and the oil layer was neutralized with caustic soda solution. The sodium sulfonates thus formed were recovered by adding ethyl alcohol, separating the alcohol layer, and then evaporating off the alcohol. This left a mixture of oil and sodium sulfonates. This was contacted with a water solution of barium chloride and, after separation of the oil layer and drying, the latter—Product C—was found to contain 6.9% barium and 2.5% sulfur.

#### EXAMPLE 7

##### *Barium triwax phenol carboxylate*

A barium salt of a triwax phenol carboxylate—Product D—was prepared by the method described in U. S. Patent 2,197,835. It was formed in an oil blend and contained 4.0% barium.

#### EXAMPLE 8

##### *Sulfurized barium triwax phenol carboxylate*

A sulfurized barium triwax phenol carboxylate—Product E—was prepared by the method described in U. S. Patent 2,256,441. It was prepared in an oil blend and analyzed to give 4% barium and 0.9% sulfur.

#### EXAMPLE 9

##### *Cobalt salt of triwax phenol carboxylate*

A cobalt salt—Product F—was prepared corresponding to the barium salt above (Product D). This salt contained 1.83% cobalt.

The following test results are provided to demonstrate the properties of mineral oils containing small amounts of oil detergents and the outstandingly superior properties of mineral oils containing small amounts of the said detergents and of the aforesaid oil-soluble, phosphorus- and sulfur-containing cycle stock-P<sub>2</sub>S<sub>5</sub> reaction products.

#### EXAMPLE 10

An accelerated oxidation test was used to determine the corrosive nature of lubricating oils on an automobile connecting rod bearing. The oil used consisting of Pennsylvania neutral and residuum stocks separately refined by means of chlorex and then blended to give an S. A. E. 20

75

grade motor oil with a specific gravity of 0.872, a flash point of 435° F., and a Saybolt Universal viscosity of 318 seconds at 100° F. The oil was tested by adding a section of a bearing containing a cadmium-silver alloy surface, weighing about 6 grams, and heating it to 175° C. for 22 hours while a stream of air was bubbled against the surface of the bearing. The loss in weight of the bearing during this treatment measures the amount of corrosion that has taken place. The results obtained in this test are set forth in Table II below.

Table II

|    | Detergent | Per cent Wt. | Stabilizer   | Per cent Wt. | Mgs. Loss in Weight |
|----|-----------|--------------|--------------|--------------|---------------------|
|    | Blank Oil |              |              |              |                     |
| 20 | Product A | 2            |              |              | 21                  |
|    | Do        | 2            | +Product Two | 1            | 0                   |
| 21 | Product B | 2            |              |              | 21                  |
|    | Do        | 2            | +Product Two | 1            | 0                   |
| 22 | Product C | 2            |              |              | 38                  |
|    | Do        | 2            | +Product Two | 1            | 0                   |
| 23 | Product D | 2            |              |              | 15                  |
|    | Do        | 2            | +Product Two | 1            | 0                   |
| 24 | Product E | 2            |              |              | 33                  |
|    | Do        | 2            | +Product Two | 1            | 1                   |
| 25 | Product F | 2            |              |              | 26                  |
|    | Do        | 2            | +Product Two | 1            | 0                   |

It will be apparent from inspection of the results presented in Table II that the blank oil is unsatisfactory in view of its corrosivity, as shown by the high milligram loss in weight of the bearing. When a detergent alone is added to the oil there is little or no improvement and, in some instances the oil is impaired. The results with Products C, E and F, for example, demonstrate that some detergents accelerate corrosion. However, when a small amount of a cycle stock-P<sub>2</sub>S<sub>5</sub> reaction product, such as Product Two, is added to the oil containing any one of the detergents, the resulting oil blends are substantially non-corrosive to bearing metals.

#### EXAMPLE 11

Tests of an oil, of oil blends containing only an oil detergent, and of oil blends containing an oil detergent and an oil-soluble, phosphorus- and sulfur-containing reaction product as defined above, were carried out to determine further the comparative behavior of the unblended oil, the oil containing only the detergent and the oil containing a detergent and said reaction product, under actual operating conditions.

In this test a single cylinder Lauson engine was operated for 36 hours with an oil temperature of 290° F. and a jacket temperature of 212° F. The oil used was a solvent-refined oil having a Saybolt Universal viscosity of 45 seconds at 210° F. (Kinematic viscosity 5.75 at 210° F.). After 36 hours the acidity, as measured by the neutralization number (N. N.), and the Kinematic viscosity of the oil were determined. The neutralization number (N. N.) rating is obtained by dividing the specific neutralization number of the oil alone which is run in the engine preceding the oil blend, by the neutralization number of the oil blend. Ratings of greater than 1 indicate that the oil blend is less acidic than the oil alone and, therefore, superior thereto; and ratings of less than 1 indicate that the oil blend is more acidic than the oil alone and, therefore, inferior thereto. Average results for the oil alone (unblended oil) are presented inasmuch as the neutralization number and kinematic viscosity of the oil alone vary slightly when samples of the same are run in the same engine; this

variation is attributed to the condition of the engine parts and other factors involved in the test. The results of these tests are set forth in Table III below.

Table III

| Detergent | Per cent Wt. | Stabilizer   | Per cent Wt. | 36 Hour Results |                 |              |
|-----------|--------------|--------------|--------------|-----------------|-----------------|--------------|
|           |              |              |              | N. N.           | K. V. @ 210° F. | N. N. Rating |
| Oil alone | (1)          | (1)          |              | 10.0            | 10.5            |              |
| Product E | 1.5          |              |              | 8.7             | 10.28           | 1.2          |
| Do.       | 1.5          | +Product Two | 1.5          | 0.9             | 6.36            | 6.5          |

<sup>1</sup> Average results.

The results in Table III indicate that a detergent oil blend, without a stabilizer, is only of the same order of effectiveness as the oil alone; whereas, an oil blend containing a detergent and a stabilizer is appreciably more effective than the oil alone or the said detergent oil blend.

## EXAMPLE 12

The effectiveness of the oil composition of this invention in actual engine tests is further demonstrated by the following results which were obtained in a Chevrolet engine. This test consisted of operating a Chevrolet engine for 36 hours at 30 brake horsepower with an oil temperature of 280° F. and a jacket temperature of 200° F. A solvent-refined oil having an S. U. V. of 65 seconds at 210° F. was used. At the end of the test, the neutralization number (N. N.) of the oil and the average weight loss of a half bearing were determined. Copper-lead bearings were used. The results, presented below in Table IV, demonstrate that the oil alone is rather unsatisfactory, and that the corrosivity thereof is substantially reduced when small amounts of a detergent and a stabilizer are incorporated therein. These test results also indicate that the corrosivity of the oil is materially counteracted by using suitable concentrations of a stabilizer with a given concentration of a detergent.

Table IV

| Detergent | Per cent Wt. | Stabilizer  | Per cent Wt. | N. N. Value | Bearing Loss, grams |
|-----------|--------------|-------------|--------------|-------------|---------------------|
| Oil alone |              |             |              |             |                     |
| Product E | 2.5          | Product Two | 0.75         | 6.5         | 1.210               |
| Do.       | 2.5          | do          | 1.5          | 4.4         | 0.960               |
|           |              |             |              | 3.7         | 0.202               |

## EXAMPLE 13

A three cylinder General Motors 3-71 Diesel engine was run at 2000 R. P. M. with an oil temperature of 230° F. and a jacket temperature of 180° F. When the air box pressure increased more than 3 inches of mercury over the original pressure, the ports were considered sufficiently closed to stop the test. In Table V below the time in hours to reach this condition is noted. A solvent refined S. A. E. 30 grade Mid-Continent oil was used in these tests.

Table V

## Hours to Port Closure

|                                     |     |
|-------------------------------------|-----|
| Oil alone                           | 122 |
| Oil+2.5% Product +0.75% Product Two | 322 |

As indicated hereinabove, preference is given herein to those oil detergents defined as metal sulfonates of wax-substituted aromatic hydro-

carbons. This preference is influenced by their outstanding pour depressing properties as illustrated below in Table VI, wherein a related oil detergent, derived from a petroleum fraction (barium salt of a petroleum oil sulfonate, Product C) is also shown for comparative purposes. The latter detergent is ineffective as a pour point depressant. The oil used in these tests was a solvent refined oil having an S. U. V. of 65 seconds at 210° F., and A. S. T. M. pour tests are reported in ° F.

Table VI

| 15 | Detergent | Conc., per cent wt. | A. S. T. M. pour test, ° F. |
|----|-----------|---------------------|-----------------------------|
|    | Product A | 1.0                 | +20                         |
| 20 | Product B | 1.0                 | -20                         |
|    | Product C | 1.0                 | -15                         |
|    |           |                     | +20                         |

The results set forth in Tables II through V demonstrate the outstanding qualities of the mineral oil compositions contemplated herein. As shown in these tables, they possess a high degree of resistance to oxidation and particularly desirable detergent properties. The results presented in Table VI above further demonstrate the superior quality of the preferred oil detergents, metal salts of wax-substituted aromatic hydrocarbon sulfonic acids, as evidenced by their pour depressant properties.

As contemplated by the present invention, concentrations of from about 0.5 per cent to about 10 per cent of an oil detergent are used in an oil fraction, but concentrations of the order of about 2 per cent have been found to be satisfactory for most purposes. The concentration of oil-soluble, phosphorus- and sulfur-containing reaction product of a cycle stock and P<sub>2</sub>S<sub>5</sub> may be varied from about 0.05 per cent to about 5.0 per cent; in general, however, about 1.0 per cent will be satisfactory.

As indicated hereinabove, the mineral oil compositions of this invention may also contain one or more other oil-soluble, phosphorus- and sulfur-containing reaction products, such as those obtained from oleyl alcohol and P<sub>2</sub>S<sub>5</sub>, and a dicyclic terpene and a phosphorus sulfide, all as defined above. Oils of excellent quality are obtained with from about 0.10 per cent to about 1.0 per cent of such a reaction product, incorporated with the aforesaid quantities of an oil detergent and of a cycle stock reaction product of the type defined above.

Mineral oil concentrates are also contemplated herein, such concentrates containing substantially larger concentrations of an oil detergent and of a cycle stock-P<sub>2</sub>S<sub>5</sub> reaction product, than those enumerated above. That is, relatively large amounts of the said materials may be incorporated in an oil fraction in which they are readily soluble, and the oil concentrate so obtained may thereafter be diluted with a suitable quantity of the said oil fraction prior to use. It is to be understood that these mineral oil concentrates may also contain one or more of the aforesaid other oil-soluble, phosphorus- and sulfur-containing reaction products, such as those obtained from oleyl alcohol or a dicyclic terpene, in amounts substantially in excess of those described above.

In preparing the mineral oil compositions and concentrates contemplated herein, an oil detergent and a cycle stock-P<sub>2</sub>S<sub>5</sub> reaction product, as

defined hereinabove, may be incorporated in a mineral oil in any one of several ways. For example, the cycle stock reaction product may be added to an oil fraction containing an oil detergent; an oil detergent may be added to the reactants (cycle stock and  $P_2S_5$ ) used in the preparation of the said reaction product and, in such case, will be present during the reaction. It is possible that the oil detergent may react with the cycle stock and  $P_2S_5$  to form a complex reaction product under the reaction conditions enumerated above; the product obtained in this manner may then be added to an oil fraction. Accordingly, it will be apparent that the mineral oil compositions and concentrates of this invention are complex in nature, for it is possible that an oil detergent and a cycle stock reaction product may be present individually in an oil fraction, or may also be present therein as a physical combination or, further, may be present therein in the form of a single chemical composition. In the same connection, it will also be apparent that an oil detergent and a reaction product of the aforesaid type may enter into chemical reaction when the oil composition is used as a lubricant under certain conditions, such for example, as a lubricant in an engine operating at relatively high temperatures.

In view of the foregoing, the term "mineral oil composition," as used herein and as recited in all of the appended claims, is inclusive of all mineral oil fractions containing an oil detergent and a cycle stock reaction product as defined above, in the concentrations recited above, and is inclusive of oil compositions obtained or prepared by any one of the aforesaid several typical procedures. Correspondingly, the term "mineral oil concentrate" is inclusive of all mineral oil fractions containing relatively large amounts of the said oil detergent and said reaction product.

It is to be understood that the examples, procedures and oil compositions described hereinabove are illustrative only and are not to be construed as limiting the scope of this invention thereto. For example, all cycle stocks as defined above may be used in place of those shown in the examples, although those shown are preferred. Also, while the sulfonates and other illustrative oil detergents are preferred of their class, all compounds coming within the aforesaid definition of an oil detergent may be used. Furthermore, the mineral oil fractions disclosed above are but typical of the fractions which may be used.

We claim:

1. An improved mineral oil composition comprising a viscous mineral oil fraction having in admixture therewith: a minor proportion, from about 0.5 per cent to about 10 per cent, of an oil-soluble salt characterized by detergent action in oil; and a minor proportion, from about 0.05 per cent to about 5.0 per cent, of an oil-soluble, phosphorus- and sulfur-containing reaction product obtained by reaction of phosphorus pentasulfide and a hydrocarbon stock at a temperature between about 125° C. and about 200° C. for a relatively short time, said hydrocarbon stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said hydrocarbon stock.

2. An improved mineral oil composition com-

prising a viscous mineral oil fraction having in admixture therewith: a minor proportion, from about 0.5 per cent to about 10 per cent, of an oil-soluble metal salt of an organic acid characterized by detergent action in oil; and a minor proportion, from about 0.05 per cent to about 5.0 per cent, of an oil-soluble, phosphorus- and sulfur-containing reaction product obtained by reaction of phosphorus pentasulfide and a hydrocarbon stock at a temperature between about 125° C. and about 200° C. for a relatively short time, said hydrocarbon stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said hydrocarbon stock.

3. An improved mineral oil composition comprising a viscous mineral oil fraction having in admixture therewith: a minor proportion, from about 0.5 per cent to about 10 per cent, of an oil-soluble metal salt of an organic acid characterized by detergent action in oil; and a minor proportion, from about 0.05 per cent to about 5.0 per cent, of an oil-soluble, phosphorus- and sulfur-containing reaction product obtained by reaction of phosphorus pentasulfide and a cycle stock at a temperature between about 125° C. and about 200° C. for a relatively short time, said cycle stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said cycle stock.

4. An improved mineral oil composition comprising a viscous mineral oil fraction having in admixture therewith: a minor proportion, from about 0.5 per cent to about 10 per cent, of an oil-soluble metal salt of an organic acid characterized by detergent action in oil; and a minor proportion, from about 0.05 per cent to about 5.0 per cent, of an oil-soluble, phosphorus- and sulfur-containing reaction product obtained by reaction of phosphorus pentasulfide and a cycle stock at about 150° C. for about four hours, said cycle stock being characterized by an olefin content of from about 3 per cent to about 7 per cent and an aromatic content of from about 40 per cent to about 60 per cent, and the said phosphorus pentasulfide representing about 5 per cent of the cycle stock.

5. An improved mineral oil composition comprising a viscous mineral oil fraction having in admixture therewith: a minor proportion, from about 0.5 per cent to about 10 per cent, of an oil-soluble metal salt of an organic acid characterized by detergent action in oil; and a minor proportion, from about 0.05 per cent to about 5.0 per cent of an oil-soluble, phosphorus- and sulfur-containing reaction product obtained by reaction of phosphorus pentasulfide and a thermal recycle stock at about 150° C. for about four hours, said thermal recycle stock being characterized by an olefin content of about 6 per cent and an aromatic content of about 47 per cent, and the said phosphorus pentasulfide representing about 5 per cent by weight of the said thermal recycle stock.

6. An improved mineral oil composition comprising a viscous mineral oil fraction having in admixture therewith: a minor proportion, from about 0.5 per cent to about 10 per cent, of an oil-

soluble metal salt of an organic acid characterized by detergent action in oil; and a minor proportion, from about 0.05 per cent to about 5.0 per cent, of an oil-soluble, phosphorus- and sulfur-containing reaction product obtained by reaction of phosphorus pentasulfide and a thermal recycle stock at about 150° C. for about four hours, said thermal recycle stock being characterized by an olefin content of about 5 per cent and an aromatic content of about 57 per cent, and the said phosphorus pentasulfide representing about 5 per cent of the said thermal recycle stock.

7. An improved mineral oil composition comprising a viscous mineral oil fraction having in admixture therewith: a minor proportion, from about 0.5 per cent to about 10 per cent, of an oil-soluble metal sulfonate; and a minor proportion, from about 0.05 per cent to about 5.0 per cent, of an oil-soluble, phosphorus- and sulfur-containing reaction product obtained by reaction of phosphorus pentasulfide and a cycle stock at a temperature between about 125° C. and about 200° C. for a relatively short time, said cycle stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said cycle stock.

8. An improved mineral oil composition comprising a viscous mineral oil fraction having in admixture therewith: a minor proportion, from about 0.5 per cent to about 10 per cent, of an oil-soluble metal salt of a wax-substituted benzene sulfonic acid; and a minor proportion, from about 0.05 per cent to about 5.0 per cent, of an oil-soluble, phosphorus- and sulfur-containing reaction product obtained by reaction of phosphorus pentasulfide and a cycle stock at a temperature between about 125° C. and about 200° C. for a relatively short time, said cycle stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said cycle stock.

9. An improved mineral oil composition comprising a viscous mineral oil fraction having in admixture therewith: a minor proportion, from about 0.5 per cent to about 10 per cent, of an oil-soluble barium salt of a diwax-substituted benzene sulfonic acid; and a minor proportion, from about 0.05 per cent to about 5.0 per cent, of an oil-soluble, phosphorus- and sulfur-containing reaction product obtained by reaction of phosphorus pentasulfide and a cycle stock at a temperature between about 125° C. and about 200° C. for a relatively short time, said cycle stock

being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said cycle stock.

10. An improved mineral oil composition comprising a viscous mineral oil fraction having in admixture therewith: a minor proportion, from about 0.5 per cent to about 10 per cent, of an oil-soluble basic barium salt of a diwax-substituted benzene sulfonic acid; and a minor proportion, from about 0.05 per cent to about 5.0 per cent, of an oil-soluble, phosphorus- and sulfur-containing reaction product obtained by reaction of phosphorus pentasulfide and a cycle stock at a temperature between about 125° C. and about 200° C. for a relatively short time, said cycle stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said cycle stock.

11. An improved mineral oil composition comprising a viscous mineral oil fraction having in admixture therewith: a minor proportion, from about 0.5 per cent to about 10 per cent, of an oil-soluble basic barium salt of a diwax-substituted naphthalene sulfonic acid; and a minor proportion, from about 0.05 per cent to about 5.0 per cent, of an oil-soluble, phosphorus- and sulfur-containing reaction product obtained by reaction of phosphorus pentasulfide and a cycle stock at a temperature between about 125° C. and about 200° C. for a relatively short time, said cycle stock being characterized by an olefin content of from about 3 per cent to about 7 per cent and an aromatic content of from about 40 per cent to about 60 per cent, and the said phosphorus pentasulfide representing from about 1 per cent to about 8 per cent by weight of the said cycle stock.

HENRY G. BERGER.  
EVERETT W. FULLER.

#### REFERENCES CITED

The following references are of record in the file of this patent:

#### UNITED STATES PATENTS

| Number    | Name                | Date          |
|-----------|---------------------|---------------|
| 2,316,082 | Loane et al. -----  | Apr. 6, 1943  |
| 2,316,083 | Loane et al. -----  | Apr. 6, 1943  |
| 2,279,086 | Bergstrom -----     | Apr. 7, 1942  |
| 2,197,835 | Reiff -----         | Apr. 23, 1940 |
| 2,373,094 | Berger et al. ----- | Apr. 10, 1945 |